

## UNITED STATES PATENT OFFICE

2,344,411

TREATMENT OF CELLULOSIC MATERIAL TO  
INCREASE ITS REACTIVITYRichard E. Reeves, Yonkers, N. Y., assignor to  
The Chemical Foundation, Incorporated, a cor-  
poration of DelawareNo Drawing. Application May 29, 1939,  
Serial No. 276,441

1 Claim. (Cl. 260—212)

This invention relates to the treatment of cellulosic material to increase its reactivity.

As those skilled in the art know, few natural chemical products have had as many speculatively assigned formulae as cellulose. At the present time, it is generally accepted, as a working hypothesis that the cellulose molecule is comprised in part of anhydroglucose residues, containing three alcoholic hydroxyl groups for every six carbon atoms.

It has been shown (Jackson and Judson J. Am. Chem. Soc. 59, 2049 (1937); 60, 989 (1938)) that both cotton and wood cellulose may be drastically oxidized by means of aqueous periodic acid to form a product which contains aldehydic groups and which product is soluble in hot water and cold dilute acids. These investigators sought to secure as complete an oxidation as possible by treating cotton, for example for a period of 430 hours with a strong solution of the acid.

10 on the fiber for various periods of time and the differentially treated samples were washed free of the acid with water. To determine the extent of oxidation and increased reactivity the samples were treated with a fuchsin-sulphurous reagent for 30 minutes to develop a purple color. This reagent consisted of 0.5% fuchsin in water to which sufficient sulphurous acid was added to completely decolorize the solution. To further determine the characteristics of the modified cellulosic material the dyed products were treated with N/10 sodium hydroxide.

15 During the course of these treatments the amount of periodic acid consumed by the fibers was determined at different intervals to thus correlate the degree of oxidation of the fibers with the ability to form a dye with the fuchsin-sulphurous acid solution. The results of treatment of this character are indicated in the following table:

Table

| Mercerized cotton fiber treated with 10 cc. of 0.125 molar periodic acid at 20°-24° C. | Time of treatment | 0.125 M. periodic acid used by sample | Coloration after 30 min. at 20° C. with fuchsin-sulphurous acid | Action of dyed product with cold N/10 sodium-hydroxide              |
|----------------------------------------------------------------------------------------|-------------------|---------------------------------------|-----------------------------------------------------------------|---------------------------------------------------------------------|
| Untreated control.....                                                                 |                   |                                       | Faint pink.....                                                 | Complete loss of color, fiber intact.                               |
| 0.128 g. cotton.....                                                                   | 15 min.....       | 0.03-0.05 cc.....                     | Magenta.....                                                    | Gradual loss of color, fiber apparently intact.                     |
| 0.1204 g. cotton.....                                                                  | 24 hrs.....       | 0.35 cc.....                          | Purple.....                                                     | Extensive loss of color and fiber disintegration, partly dissolved. |
| 0.122 g. cotton.....                                                                   | 4 days.....       | 0.86 cc.....                          | Purple-black.....                                               | Dissolved completely with loss of color.                            |
| 0.128 g. cotton.....                                                                   | 9 days.....       | 1.32 cc.....                          | do.....                                                         | Do.                                                                 |

The major purpose of these investigations evidently was to correlate the chemical structure of starch and cellulose.

It has now been discovered that the chemical reactivity of cellulose may markedly be modified by a controlled or selective oxidation. Such modification has profound technological significance the extent or scope of which is illustrated didactically herein in respect to dyeing or dye acceptance of cellulosic fabrics.

It has been found that if cellulosic material, for example mercerized cotton fibers, is treated with relatively dilute periodic acid at moderate temperature new properties are imparted to the material particularly in respect to its action toward dyes.

The type of treatment to be given the fibers under the invention is illustrated by the following example:

## EXAMPLE I

0.12 g. samples of mercerized cotton fibers were treated with 10 cc. portions of 0.12 molar periodic acid at 20°-24° C. The acid was allowed to act

35 As will be observed from inspection of the table, treatment of the control (mercerized cotton) with the dye solution produced but a faint coloration. Treatment of the dyed control with N/10 sodium hydroxide completely destroyed the color. However, when a similar sample of mercerized cotton fiber was treated for 15 minutes with the indicated dilute solution of periodic acid the dyeing was considerably enhanced, the dyed fabric being of a deeper color. It is particularly 40 to be observed that such dye is apparently much more stable than that combined with the untreated control, for an equivalent treatment with the caustic solution effected less loss in color with no apparent attack on the cellulose fibers themselves.

45 The degree of oxidation of the cellulosic material by the periodic acid must be maintained within close if not critical limits in order to secure the desired improvement in reactivity. As will be observed from the table, as the time of treatment with the periodic acid is increased the absorbability of the fiber for the dye measurably increases as is indicated by the marked

increase in depth of the color. However, such prolonged treatments are too drastic, for the fibers so treated, when immersed in the cold caustic solution not only completely lost color but the fibers themselves were partly or completely dissolved.

In order to determine the commercial feasibility of the treatment, a number of other experiments were conducted. It was found that preliminary treatment of cellulosic material, particularly cotton fibers with periodic acid under conditions controlled short of complete oxidation insured the production of a cellulosic material of new characteristics. This treatment renders the cellulosic material potentially reactive, so to speak, as is clearly indicated by its acceptance of typical dyes. It was obvious that the preliminary mild treatment with 0.15 M. periodic acid markedly improves the amenability of the fabric to dyeing. For example, the preliminarily treated material dyed with fuchsin-sulphurous acid solution develops a deep purple, whereas an untreated sample of the same fabric develops but a faint pink. This same marked differential in dye acceptance and resulting color gradation obtains similarly when other dyes are employed as for example, o-tolyl hydrazene and p-nitro phenyl hydrazine.

As will be appreciated, the mechanism of this reaction is difficult precisely to explain. It is possible that the marked increase in reactivity of the cellulose is due to a selective oxidation of one or more of the alcoholic hydroxyl groups, conceivably those at positions 2 and 3. Whatever may be the action taking place, it is a fact that it is highly specific or critical, both as to degree or time of treatment and as to the reactant employed. It has been found, for example, that treatment of cellulosic material with equivalent amounts of perchloric acid will not impart the same increased reactivity to cellulose which is effected by treatment with periodic acid.

While periodic acid has been described herein as the preferred treating agent, it is to be understood that this is also intended to include its equivalents, i. e. its salts, such as the sodium salt

of the acid. When salts are used in lieu of the acid the optimum pH may be attained by utilizing a suitable mineral acid.

It will be appreciated that this type of treatment is of marked utility and has many ramifications in the art. The particular examples described herein serve effectively to illustrate the modification of the chemical activity of cellulosic material as a result of the invention. The treatment obviously has direct and immediate utility for the purpose of enhancing the dye acceptance of cellulosic fabrics. However, the treatment may be employed in any circumstance in which cellulose is involved, especially as a chemically reacting component. For example, the invention may be utilized in the plastic industry to produce new and improved forms of cellulose containing synthetic resins. The cellulosic starting material, such as cotton and other cellulosic fibers, after any desired preliminary treatment may be treated according to the invention, that is to say, with periodic acid solutions of controlled strength and for predetermined periods of time, so as to oxidize or otherwise chemically modify the cellulose molecule. Thereafter the modified cellulose containing aldehydic groupings may be reacted with phenol so as to effect a condensation reaction through the aldehydic linkage. Thereafter the initial condensation product may be submitted to treatments known in the art to produce the various modified forms of the resin.

It will therefore be understood that while particular treatments are described herein by way of examples, these are given to illustrate the broader concept of the invention, namely, the modification of the cellulosic material to increase its chemical reactivity.

**I claim:**

40 A method of modifying the chemical characteristics of cellulose, which comprises, subjecting the cellulose to the action of a 0.12-0.15 M. periodic acid solution, at room temperature for a period of less than 24 hours, to secure only partial oxidation of the cellulose.

RICHARD E. REEVES.